

## UNITED STATES PATENT OFFICE

2,108,125

CELLULOSE PRODUCTS AND METHOD OF  
MAKING

Samuel Isaac Hoddeson, New Brunswick, N. J.,  
and Roy Mackay Meiklejohn, New York, N. Y.,  
assignors to General Chemical Company, New  
York, N. Y., a corporation of New York

No Drawing. Application December 5, 1935,  
Serial No. 53,002

11 Claims. (Cl. 260—146)

This invention relates in general to low viscosity cellulose products and their manufacture. It is particularly directed to a method of treating cellulose to prepare an initial material which 5 may be nitrated to yield directly low viscosity nitrocellulose products.

The invention further comprehends low viscosity cellulose as a new article of manufacture.

The development of the nitrocellulose lacquer 10 or varnish industry has, in the past, been greatly impeded because of the high viscosity of solutions containing even a small proportion of nitrated cellulose of the "laquer" or  $12\% \pm .50\%$  nitrogen type. This has retarded the general 15 commercial application of such derivatives in the industry since highly viscous products when dissolved or thinned to a usable consistency carry an insufficient quantity of film-forming ingredient to yield a film or coating of substantial 20 thickness in one application. Hence numerous successive applications are required.

While the viscosity of cellulose has in the past 25 been varied over a wide range, it has not been possible, as far as we are aware, to prepare a cellulose of sufficiently low viscosity so that a nitrated cellulose suitable for commercial use in lacquers or varnishes could be prepared directly therefrom. Accordingly it has been the practice 30 to nitrate a cellulose and thereafter to subject the nitrated cellulose to an aftertreatment for reducing its viscosity to within an appropriate range. In this manner it has been possible to obtain nitrated cellulose products of sufficiently 35 low viscosity for commercial use in lacquers, paints, varnishes, etc. However, the aftertreatment of nitrated cellulose presents numerous objections. Chemical treatments result in reduced yields and produce a product difficult to bleach 40 to a satisfactory color. Treatment in water suspension under pressure presents a serious explosion hazard unless equipment is designed to minimize this danger, and this involves additional expense for equipment and operation.

45 It will be evident, therefore, that a cellulose that may be nitrated to yield directly low viscosity products constitutes a substantial advance in the art.

It is known that celluloses such as cotton and 50 wood pulp may be purified by treatment with alkaline liquors, and digestion in weakly alkaline solutions is a customary step in the preparation of cotton for nitration. That such procedures could be manipulated to yield cellulose from 55 which low viscosity ( $\frac{1}{2}$  second) products could

be obtained directly upon nitration was not formerly known.

In accordance with the present invention, it has been discovered that extremely low viscosity cellulose of high alpha- beta-cellulose content 5 (i. e. about 98% or more insoluble as determined by the usual soda-soluble test for gamma cellulose) may be obtained from ordinary cellulose such as cotton, or wood cellulose by employing a series of treatments wherein the cellulose is 10 first treated with a dilute alkaline solution, then mercerized, and subsequently digested in weakly alkaline solution. Furthermore, the low viscosity of the cellulose has been found to inure to the benefit of nitrated cellulose prepared therefrom 15 so that by utilizing nitration methods commonly employed a nitrated cellulose (11%—12.8% nitrogen) of low viscosity is obtained which may be employed directly without further reduction in viscosity for the preparation of nitrocellulose 20 lacquers, varnishes, etc. of high concentration.

The process of the present invention is especially applicable to cotton linters, which constitute the usual "raw material" for the preparation of nitrated cellulose. It is also applicable to treatment of cellulose from other sources, cotton 25 cellulose or alpha cellulose derived from wood, bagasse, or other vegetable origin to yield products of correspondingly reduced viscosity.

Cotton linters are purified by the preliminary 30 alkaline digestion with the result that the subsequent mercerization liquid may effectively penetrate the fibers, thus fats, oils, waxes, and any remnants of hulls are removed in the first step. The mercerization serves to effect an important reduction of viscosity of the cellulose and at the same time appears to render the cellulose molecule susceptible to further viscosity reduction by subsequent alkaline digestion. Sodium hydroxide or other alkali metal or alkaline earth 35 compounds may be employed as the alkaline reagent. Thus KOH and the salts of sodium and potassium, such as the carbonates, sulfides, sulfites, phosphates, and silicates may be employed but the larger quantities required and/or 40 the high prices of most of these reagents render their use less economical than the use of caustic soda.

The results will vary with conditions of treatment and in order to secure the most satisfactory products the initial material, such as cotton linters or refined wood pulp, may be digested for 3 to 15 hours at a temperature of  $150^{\circ}$  to  $200^{\circ}$  C. (under a pressure of 60 to 150 pounds per 50 square inch) in a solution having a hydroxyl ion 55

concentration equivalent to a solution containing .25% to 4.0% of NaOH. This serves to reduce the viscosity of the cellulose in terms of the viscosity of nitrocellulose producible therefrom from as much as several thousand to between about 100 and about 1700. The treatment is preferably regulated to yield a viscosity of 100 to 300 seconds. The treated cellulose is then mercerized, for example by immersion in an aqueous solution having a hydroxyl ion concentration equivalent to a solution containing 14% to 28% NaOH maintained at 2° to 32° C. (35° to 90° F.) for a period of 3 minutes to an hour. The mercerization preferably is regulated to further reduce the viscosity to between about 15 and about 60 seconds. The cellulose, after mercerization, is then again digested at a temperature of 150° to 200° C. (under a pressure of 60 to 150 pounds per square inch) for a period from 3 to 24 hours in an aqueous solution of .25% to 3.0% NaOH or equivalent solution. This digestion serves to reduce the viscosity to that corresponding to  $\frac{1}{2}$  second nitrocellulose.

After each treatment of the cellulose the excess alkaline solution is drained off and preferably the cellulose is washed well with water and centrifuged prior to subsequent treatment.

The customary method of measuring the viscosity of cellulose comprises determining the viscosity of a solution of 2.5 grams of the dried cellulose in 97 cc. of cuprammonium solvent (an aqueous solution containing  $30 \pm 0.5$  grams copper,  $165 \pm 2.0$  grams NH<sub>3</sub>, and 10 grams of sucrose per liter), referred to as " $\frac{1}{2}$  concentration".

As far as we are aware no cellulose has been offered to the trade or produced prior to the present invention which has a viscosity below 3 seconds when dissolved in  $\frac{1}{2}$  concentration standard cuprammonium solution. A cellulose exhibiting a viscosity of 3 seconds in  $\frac{1}{2}$  concentration solution, upon nitration in the customary manner so as to obtain commercial yields, gives a nitrated cellulose of approximately 15 to 20 seconds viscosity in a 12.2% solution of standard viscosity solvent, e. g. the solvent known to the trade as "366" (20% ethyl acetate of 85-88% ester content, 25% denatured alcohol 2B, 55% toluol).

Half second viscosity nitrocellulose has a viscosity in 20% solution (20%—dry basis—nitrocellulose in standard solvent) of from 2 to 5 seconds, equivalent to  $\frac{1}{2}$  second in 12.2% solution. Viscosity determinations of products of half second viscosity are customarily made in 20% solution for ease of manipulation.

In view of the low viscosity of the cellulose products of the present invention the customary methods of viscosity determination are not directly applicable.

The reason for lack of direct measurement of the cellulose resides in the fact that the viscosity of the full strength solution of cellulose in cuprammonia is so much lower than the viscosity of the 20% strength of nitrocellulose that the standard falling ball method can not be applied to the cuprammonia solution. Neither can the cellulose concentration be increased since the cuprammonia solution is not capable of dissolving any appreciable excess over the standard 5 grams of cellulose.

In order, therefore, to establish a direct relationship between the viscosity of a cellulose and the nitrocellulose produced therefrom, and provide a method of determining viscosity that can be applied directly to the cellulose, a different

method has been utilized which consists in measuring the time required to empty a No. 7 pipette of 50 c. c. capacity. This pipette requires seven seconds to discharge 50 c. c. of water at 25° C. A tabulation is set forth below showing the relative viscosity of a full strength solution of cellulose in cuprammonia solution and of the nitrocellulose produced from same at 20% concentration.

| 20% concentration nitrocellulose viscosity | Equivalent 12.2% concentration nitrocellulose viscosity | Full strength cuprammonia solution  |                                        | 15   |
|--------------------------------------------|---------------------------------------------------------|-------------------------------------|----------------------------------------|------|
|                                            |                                                         | Viscosity pipette method #7 pipette | Viscosity standard falling ball method |      |
| Seconds                                    | Seconds                                                 | Seconds                             | Seconds                                |      |
| 2.0                                        | 11.0                                                    | 11.0                                | 11.0                                   |      |
| 2.2                                        | 11.4                                                    | 11.4                                | 11.4                                   |      |
| 2.6                                        | 11.6                                                    | 11.6                                | 11.6                                   | 20   |
| 2.8                                        | 11.6                                                    | 11.6                                | 11.6                                   |      |
| 3.4                                        | 12.0                                                    | 12.0                                | 12.0                                   |      |
| 4.2                                        | 12.4                                                    | 12.4                                | 12.4                                   |      |
| 4.4                                        | 13.0                                                    | 13.0                                | 13.0                                   |      |
| 5.0                                        | 13.0                                                    | 13.0                                | 13.0                                   |      |
| 5.4                                        | 13.6                                                    | 13.6                                | 13.6                                   |      |
| 7.8                                        | 15.0                                                    | 15.0                                | 15.0                                   |      |
| 9.2                                        | 14.4                                                    | 14.4                                | 14.4                                   | 25   |
| 14.6                                       | 16.6                                                    | 16.6                                | 16.6                                   |      |
| 19.8                                       | 17.2                                                    | 17.2                                | 17.2                                   |      |
| 44.6                                       | 32.2                                                    | 32.2                                | 32.2                                   | 2.6  |
| 124.2                                      | 43.4                                                    | 43.4                                | 43.4                                   | 3.2  |
| 168.0                                      | 53.2                                                    | 53.2                                | 53.2                                   | 4.0  |
| 194.0                                      | 65.2                                                    | 65.2                                | 65.2                                   | 4.8  |
| 326.0                                      | 100.4                                                   | 100.4                               | 100.4                                  | 8.0  |
| 520.0                                      | 147.6                                                   | 147.6                               | 147.6                                  | 11.8 |
|                                            |                                                         |                                     |                                        | 30   |

This tabulation covering 19 samples extends over the range of 2 seconds to 520 seconds for the 20% concentration of nitrocellulose and it will be noted that for the direct preparation of " $\frac{1}{2}$  second" nitrocellulose (between 2 and 5 seconds in 20% concentration) a cellulose is required whose full strength cuprammonia solution has a viscosity between 11 and 13 seconds by the pipette discharge method. On the other hand, a cellulose whose full strength cuprammonia solution has a viscosity of 2.6 seconds by the standard falling ball method has a viscosity of 32.2 seconds by the pipette discharge method or, in other words, requires nearly three times as long to discharge as does the cellulose suitable for direct preparation of " $\frac{1}{2}$  second" nitrocellulose, and the 20% solution of nitrocellulose directly prepared from this "2.6 second" cellulose has a viscosity of 44.6 seconds.

The following examples will serve to illustrate the process of the present invention.

*Example 1.*—100 parts of raw cotton linters were mixed with 1100 parts of a 1% aqueous sodium hydroxide solution and heated in a digester at a temperature of about 170° C. (100 pounds per square inch pressure) for three hours. The treated cellulose was then separated from the dilute caustic solution, washed with water, and treated with 1500 parts of an aqueous 18% sodium hydroxide solution maintained at a temperature of about 13° to 14° C. (56° F.) for 15 minutes. The mercerized cellulose was separated from the mercerization lye, washed with water, and heated with 1100 parts of aqueous 2% sodium hydroxide solution for nine hours at a temperature of about 170° C. The product, which comprised more than 98% alpha-beta cellulose, was then washed thoroughly with water. The washed cellulose product, when nitrated under standard conditions with the usual nitrating acid mixture yielded a (12%  $\pm$  .5% nitrogen) nitrocellulose product having a viscosity of 4.2 seconds when tested in a 20% solution; i. e. the

nitrated cellulose product was what is known as  $\frac{1}{2}$  second nitrocellulose.

*Example 2.*—100 parts of raw cotton linters were heated with 1100 parts of aqueous .75% sodium hydroxide solution at 170° C. for 16 hours. The treated linters were then separated from the sodium hydroxide solution, washed with water, and mercerized for 15 minutes in 1500 parts of an aqueous 18.25% sodium hydroxide solution maintained at around 12° to 14° C. (53° to 57° F.). The treated cellulose was then separated from the mercerization lye, washed with water, and digested for six hours in 1100 parts of aqueous 2% sodium hydroxide solution at a temperature of 170° C. After this treatment the cotton linters were thoroughly washed with water and nitrated in the customary manner. The nitrocellulose product possessed a viscosity of 4.6 seconds in 20% solution.

*Example 3.*—100 parts of bleached sulfite wood pulp (about 85% alpha cellulose) were mixed with 1100 parts aqueous .75% sodium hydroxide solution and heated at a temperature of about 170° C. (100 pounds per square inch pressure) for a period of five hours. The treated pulp was then separated from alkaline solution, washed with water, and treated with 1500 parts of aqueous 18.6% sodium hydroxide solution for one hour at a temperature of about 22° C. (71° to 72° F.). The mercerized pulp was washed with water to remove the concentrated caustic and was digested with 1100 parts aqueous 1.0% sodium hydroxide solution at a temperature of 170° C. for a period of about 16 hours. This cellulose product, when nitrated in the usual manner, yielded a nitrated cellulose having a viscosity of 2.6 seconds in 20% solution.

*Example 4.*—100 parts of unbleached sulfite wood pulp were digested with 1100 parts of an aqueous solution containing 0.5% sodium hydroxide and 0.5% sodium sulfite ( $\text{Na}_2\text{SO}_3 \cdot 7\text{H}_2\text{O}$ ) at a temperature of about 170° C. for five hours. The product was separated from alkaline solution, washed with water, and mercerized with 1500 parts of an aqueous 18.4% sodium hydroxide solution for one hour at a temperature of about 22° C. (71° F.). The mercerized pulp was washed with water and digested for 16 hours at a temperature of about 170° C. in 1100 parts of aqueous 1% sodium hydroxide solution. The product was then washed to remove alkaline solution. This product, upon nitration, yielded a nitrated cellulose having a viscosity of 4.2 seconds in a 20% solution.

*Example 5.*—100 parts of unbleached sulfite wood pulp were digested for five hours at about 170° C. (100 pounds per square inch pressure) in 1100 parts of an aqueous 1% sodium sulfite ( $\text{Na}_2\text{SO}_3 \cdot 7\text{H}_2\text{O}$ ) solution, the digested pulp was then separated from sodium sulfite solution and washed with water. The washed pulp was mercerized with 1500 parts of an aqueous 18.4% sodium hydroxide solution for one hour at a temperature of 22° C. (71° F.). The mercerized pulp was washed with water and digested for 16 hours in 1100 parts of aqueous 1% sodium hydroxide solution at a temperature of 170° C. The product was then washed as in the preceding examples. The cellulose of this treatment, upon nitration, yielded a nitrocellulose having a viscosity of 3 seconds in a 20% solution.

*Example 6.*—100 parts of wood pulp, refined by the soda process, were digested for five hours at a temperature of 170° C. with 1100 parts of an aqueous 0.75% sodium hydroxide solution. The

digested pulp was washed with water and mercerized for one hour with 1500 parts of aqueous 18.6% sodium hydroxide solution at a temperature of 22° C. (71° to 72° F.). It was then washed to remove the concentrated caustic and digested with 1100 parts of aqueous 1% sodium hydroxide solution for 16 hours at about 170° C. Upon nitration in the usual manner this product yielded a nitrocellulose having a viscosity of 0.8 second in 20% solution.

*Example 7.*—A kraft wood pulp was digested for five hours with 1100% of its weight of aqueous 0.75% sodium hydroxide solution at a temperature above 170° C. The digested pulp product was washed with water and mercerized in 1500 parts of 18.6% sodium hydroxide solution for a period of one hour at a temperature of about 22° C. It was then washed with water and redigested this time for a period of 16 hours in 1100 parts of a 1% sodium hydroxide solution at 20 a temperature of about 170° C. This cellulose, when nitrated under standard conditions and with a nitrating acid normally used in the nitrating industry, gave a nitrocellulose having a viscosity of two seconds in 20% solution.

The amounts of solutions employed in the three steps of the process are not critical but may be between 4 and 20 times the weight of the cellulose with highly satisfactory results.

The following example will serve to illustrate the usual nitration processes by which low viscosity nitrocellulose products may be prepared from the cellulose of the present invention. It is to be understood of course that any of the well-known nitration methods yield nitrocelluloses of similarly low viscosity.

*Example 8.*—The processed cellulose is picked and dried to a moisture content not to exceed 1%. 100 parts of the dried cellulose are then nitrated with 5000 parts of mixed acid containing approximately 21% to 22%  $\text{HNO}_3$ , 60% to 61%  $\text{H}_2\text{SO}_4$ , and 17% to 19%  $\text{H}_2\text{O}$ . The nitration is carried out for 25 to 30 minutes at a temperature of 35° to 40° C. The resulting nitrocellulose is then washed with water and stabilized by boiling in a final aqueous wash having an acidity between .2% and .4% (calculated as  $\text{H}_2\text{SO}_4$ ). The product represents 140 to 150 parts of nitrocellulose (dry basis), having a nitrogen content of from 11.7% to 12.1% and a viscosity in 20% solution of special solvent No. 366 within the 2 to 5 second range.

After stabilization the nitrocellulose is de-watered either in a filter press or centrifuge and then dehydrated with ethyl alcohol or other suitable dehydrating agent in order to remove all water which is objectionable in the preparation of lacquers, artificial leather, etc. It is then packaged in containers in an alcohol wet condition, the product for storage and transportation containing approximately 30% alcohol and 70% nitrocellulose.

In the above examples proportions are expressed in parts by weight.

We claim:

1. The method of preparing from cellulose fibers low viscosity cellulose, which directly on nitration by the method herein described yields a nitrocellulose of  $\frac{1}{2}$  second viscosity, which comprises removing non-cellulosic materials from the cellulose fibers, subjecting the resultant product to mercerization, and thereafter subjecting the mercerized cellulose to the action of a dilute alkaline solution having an alkalinity equal to at least  $\frac{1}{4}$  % of caustic alkali at a temperature be-

tween about 150° C. and about 200° C. for between about 3 and about 24 hours.

2. The method of preparing from cellulose fibers low viscosity cellulose, which directly on nitration by the method herein described yields a nitrocellulose of  $\frac{1}{2}$  second viscosity, which comprises treating the cellulose fibers with a dilute alkaline solution, subjecting the resultant product to mercerization, and thereafter subjecting the 10 mercerized cellulose to the action of a dilute alkaline solution having an alkalinity equal to at least  $\frac{1}{4}$  % of caustic alkali at a temperature between about 150° C. and about 200° C. for between about 3 and about 24 hours.

15 3. The method of preparing from cotton low viscosity cellulose, which directly on nitration by the method herein described yields a nitrocellulose of  $\frac{1}{2}$  second viscosity, which comprises removing oils, waxes, fats, and hulls from the cotton cellulose, subjecting the cellulose to mercerization, and thereafter subjecting the mercerized cellulose to the action of a dilute alkaline solution having an alkalinity equal to at least  $\frac{1}{4}$  % of caustic alkali at a temperature of about 170° C. 20 for between about 3 and about 24 hours.

4. The method of preparing low viscosity cellulose, which directly on nitration by the method herein described yields a nitrocellulose of  $\frac{1}{2}$  second viscosity, which comprises treating cellulose 30 with an alkaline solution corresponding to an aqueous solution containing between about  $\frac{1}{4}$  % and about 4% NaOH at a temperature between about 150° C. and about 200° C. for between about 3 and about 15 hours, mercerizing the product, and treating the mercerized product with an alkaline solution corresponding to an aqueous solution containing between about  $\frac{1}{4}$  % and about 3% NaOH at a temperature between about 150° 35 and about 200° C. for between about 3 and about 40 24 hours.

5. The method of preparing from cotton, which has been freed from oils, waxes, fats, and hulls, low viscosity cellulose, which directly on nitration by the method herein described yields a nitrocellulose of  $\frac{1}{2}$  second viscosity, which method comprises treating cotton thus purified with an aqueous solution containing between about 14% and about 28% sodium hydroxide at a temperature between about 2° and about 32° C. for between about 3 and about 60 minutes, and heating the resultant cellulose product with an aqueous solution containing between about  $\frac{1}{4}$  % and about 3% sodium hydroxide at a temperature of about 170° C. for between about 3 and about 24 hours.

55 6. The method of preparing low viscosity cellulose, which directly on nitration by the method herein described yields a nitrocellulose of  $\frac{1}{2}$  second viscosity, which comprises treating cellulose with an aqueous solution containing between about  $\frac{1}{4}$  % and about 4% of sodium hydroxide at a temperature between about 150° and about 200° C. for between about 3 and about 15 hours, treating the product with an aqueous solution containing between about 14% and about 28% sodium hydroxide at a temperature between about 2° and about 32° C. for between about 3 and about 60 minutes, and heating the resultant cellulose product with an aqueous solution containing between about  $\frac{1}{4}$  % and about 3% sodium hydroxide at a temperature of about 170° C. for between about 3 and about 24 hours.

7. The method of preparing from raw cotton linters low viscosity cellulose, which directly on nitration by the method herein described yields a nitrocellulose of  $\frac{1}{2}$  second viscosity, which comprises treating the cotton linters with an aqueous solution containing between about  $\frac{1}{4}$  % and about 4% of sodium hydroxide at a temperature between about 150° and about 200° C. for between about 3 and about 15 hours, treating the product with an aqueous solution containing between about 14% and about 28% sodium hydroxide at a temperature between about 2° and about 32° C. for between about 3 and about 60 minutes, and heating the resultant cellulose product with an aqueous solution containing between about  $\frac{1}{4}$  % and about 3% sodium hydroxide at a temperature of about 170° C. for between about 3 and about 24 hours.

8. The method of preparing from cellulose fibers low viscosity nitrocellulose of the  $\frac{1}{2}$  second type, which comprises removing non-cellulosic materials from the cellulose fibers, subjecting the resultant product to mercerization, thereafter subjecting the mercerized cellulose to the action of a dilute alkaline solution having an alkalinity equal to at least  $\frac{1}{4}$  % of caustic alkali at a temperature of about 170° C. for between about 3 and about 24 hours, and nitrating the resultant product.

9. The method of preparing from cellulose fibers low viscosity nitrocellulose of the  $\frac{1}{2}$  second type, which comprises treating the cellulose fibers with a dilute alkaline solution, subjecting the resultant product to mercerization, thereafter subjecting the mercerized cellulose to the action of a dilute alkaline solution having an alkalinity equal to at least  $\frac{1}{4}$  % of caustic alkali at a temperature between about 150° and about 200° C. for between about 3 and about 24 hours, and nitrating the resultant product.

40 10. The method of preparing from cotton low viscosity nitrocellulose of the  $\frac{1}{2}$  second type, which comprises removing oils, waxes, fats, and hulls from the cotton cellulose, subjecting the cellulose to mercerization, thereafter subjecting the mercerized cellulose to the action of a dilute alkaline solution having an alkalinity equal to at least  $\frac{1}{4}$  % of caustic alkali at a temperature of about 170° C. for between about 3 and about 24 hours, and nitrating the resultant product.

50 11. The method of preparing from raw cotton linters low viscosity nitrocellulose of the  $\frac{1}{2}$  second type, which comprises treating the cotton linters with an aqueous solution containing between about  $\frac{1}{4}$  % and about 4% of sodium hydroxide at a temperature between about 150° and about 200° C. for between about 3 and about 15 hours, treating the product with an aqueous solution containing between about 14% and about 28% sodium hydroxide at a temperature between about 2° and about 32° C. for between about 3 and about 60 minutes, heating the resultant cellulose product with an aqueous solution containing between about  $\frac{1}{4}$  % and about 3% sodium hydroxide at a temperature of about 170° C. for between about 3 and about 24 hours, and nitrating the resultant product.